

## UNITED STATES PATENT OFFICE

AUGUSTUS B. KINZEL, OF BAYSIDE, NEW YORK, ASSIGNOR TO ELECTRO METALLURGICAL CO., A CORPORATION OF WEST VIRGINIA

## HARDENING PROCESS

No Drawing.

Application filed June 27, 1928. Serial No. 288,816.

My invention relates to hardening processes for ferrous materials, and particularly to a nitrification case hardening process. It has for one of its objects the provision of a hard nitrification case in a minimum length of time, and for another, the provision of a new nitrification case hardening process, and a new material for the operation thereof.

It has been found that by the diffusion of active nitrogen at relatively low temperatures into and through a surface layer of a ferrous material object having certain alloy constituents, a hard and durable case or surface layer is obtained. This process is desirably carried out at temperatures below about 600° C., and is customarily done by heating the metal part to the appropriate temperature in an atmosphere of gaseous ammonia, over a period of time, ranging 20 from 24 hours to 90 hours.

My invention provides a new means and process for producing a harder, tougher and more ductile nitrification case upon a ferrous object in a much shorter period of time.

In practicing my invention I provide a molten nitrification bath as distinguished from the prior art which provided the nitrogen from a gaseous atmosphere. I provide preferably a molten bath of the mixed cyanides of sodium and potassium, having such a composition that a low melting point is obtained. I then immerse the object to be case hardened within the molten mixed cyanides, being careful to keep the temperature 35 below 580° C. The case hardening proceeds rapidly and in about 2 hours may produce a hardened nitride case having a thickness of about 0.001 inches.

It may be noted that this is a broadly different process from prior methods of case hardening with cyanide baths in which a temperature well above 700° C., is always reached, and a carburization case only is produced. In the process of my invention no carburization occurs at the low temperature but only a nitrification.

The resulting case obtained by the process of my invention is substantially harder than the case obtained by the prior nitrification process, and is also more ductile. When pro-

duced upon a given suitable alloy, it has a hardness about four times as great as that produced by the previous nitrification process upon the same alloy, and it is also sufficiently ductile to permit of considerable distortion, since pressure by a point or small ball upon the treated object does not crack or shatter the case hardened coating as occurs with nitrification cases produced by the methods of the prior art, which are much less resistant to deformation and pressure.

In the preparation of the case hardening bath of my invention, I find it convenient to provide a mixture of about 53% of sodium cyanide and about 47% of potassium cyanide, this mixture producing the eutectic, or lowest melting composition and fusing at about 445° C. This bath is thus fluid over a convenient temperature range below the critical point at 580° C., at which transformation 70 of the nitrification product begins to occur.

By the process as above described I am thus enabled to treat a ferrous object for case hardening to obtain a new and useful product with a saving of time, and cost. The 75 process is particularly advantageous because of the low temperature at which it operates whereby the object may be given suitable heat treatments for the production of desired physical characteristics and may thereafter be case hardened without change in the characteristics of the body or danger of deformation or internal strains. Likewise a casting of maximum hardness is obtained without the necessity for any subsequent heat treating 85 steps to temper the case.

As a bath for the operation of the process of my invention I have, above, disclosed a mixture of sodium and potassium cyanide. It is not however, necessary that such a mixture 90 be used since there are various other mixtures which obtain a similar result. For instance, mixtures of other cyanides such as sodium cyanide and zinc cyanide, or potassium cyanide and magnesium cyanide, or vice versa, 95 produce eutectic mixtures having melting points sufficiently low to be useable for the process of my invention. Alternatively, other substances than cyanide may be used, such for instance, as a mixture of a convenient 100

cyanide and a cyanamide. Likewise other salts which produce the desired reduction in melting point may be used although it is preferable that substances which evolve oxygen be excluded.

The process of my invention is particularly applicable to alloy steels, such as those containing vanadium or aluminum, as well as such elements as manganese, silicon and chromium, and such alloy steels are the preferred materials for treatment by my process. The alloys containing the vanadium and aluminum produce cases having a maximum hardness and may be made sufficiently hard to scratch glass readily. The alloys containing manganese, silicon and chromium, also produce a substantial degree of hardness although less than the first two mentioned alloying elements when treated by the process of my invention. In each case however, a substantial gain in hardness and ductility appears over a nitrified case made according to the prior art.

The hardness obtained by the process of my invention is conveniently indicated by measurements, in terms of microcharacter units, as made upon a suitable steel. Comparison was made between the hardness obtained by the previously used gaseous ammonia nitration process, and by the process of my invention, upon four typical steels having the following alloy contents, with low carbon values.

Steel No. 1— $\frac{1}{2}\%$  aluminum.

Steel No. 2— $\frac{1}{2}\%$  chromium and  $\frac{1}{2}\%$  vanadium.

Steel No. 3— $\frac{1}{2}\%$  vanadium.

Steel No. 4— $\frac{1}{2}\%$  vanadium,  $\frac{1}{2}\%$  aluminum,  $\frac{1}{4}\%$  molybdenum.

Upon hardening in gaseous ammonia, samples of these steels showed degrees of surface hardness varying between 100,000 and 300,000 microcharacter units. Samples of the same steels treated in the bath of my invention gave surface hardness values varying from 600,000 to 800,000 microcharacter units.

By the process of my invention I have thus produced a new and simple means of obtaining a case hardened surface upon ferrous objects, which is much simpler to operate, and much more rapid and effective than the previous methods.

While I have described several embodiments of the process of my invention it is capable of still other embodiments, adaptations and modifications without departure from the spirit thereof and I desire therefore that only such limitations shall be imposed upon the appended claims as are indicated therein, or required by the prior art.

I claim as my invention:

1. The process of case-hardening ferrous articles which comprises treating an article having a surface composition adapting it for

nitride casing, with a liquid non-oxidizing nitrogen-containing salt at a temperature below 600° C.

2. The process of case-hardening ferrous articles which comprises treating an article having a surface composition adapting it for nitride casing with a liquid cyanide at a temperature below 600° C. 70

3. The process of case-hardening ferrous articles which comprises treating an article having a surface containing vanadium and of a composition adapting it for nitride casing with a liquid cyanide at a temperature between 445° C. and 600° C. 75

In testimony whereof, I affix my signature. 80  
AUGUSTUS B. KINZEL.

85

90

95

100

105

110

115

120

125

130